

## United States Patent Office

3,351,556

Patented Nov. 7, 1967

1

3,351,556

METHODS AND COMPOSITIONS FOR  
STRIPPING NICKEL

Harry K. Tsourmas, North Haven, Conn., assignor to  
MacDermid, Incorporated, Waterbury, Conn., a corpora-  
tion of Connecticut  
No Drawing, Filed Mar. 24, 1965, Ser. No. 442,506  
12 Claims. (Cl. 252—102)

## ABSTRACT OF THE DISCLOSURE

Compositions and aqueous solutions thereof for strip-  
ping nickel coatings from substrates, particularly where  
copper or copper alloys are present in the substrate. The  
composition comprises generally the combination of an  
oxidizer consisting of an oxy-halogen compound of the  
group comprising specifically the chlorites, hypochlorites,  
bromates and hypobromites; a nickel complexing agent of  
the group comprising ammonia, the ammonium ion,  
amines and other known nickel complexers; a divalent  
sulfur ion-supplying compound, either organic or inor-  
ganic, as a nickel activator; and, where necessary to pre-  
vent poisoning of the stripping solution by the presence of  
copper, an organic sulfur ion-supplying compound if the  
nickel activator is not of such type or present in sufficient  
amount.

This invention relates to dissolving nickel from a sub-  
strate on which it has been plated, and is more particu-  
larly directed to compositions for and methods of stripping  
nickel deposits from ferrous metals where copper or cop-  
per alloys may or may not be present. The invention is also  
useful in stripping nickel from organic, i.e. plastic, or in-  
organic, i.e. ceramic, substrates.

Fabricated articles incorporating a plating of nickel  
sometimes fail to pass inspection because of defects in  
the plate. The reclaiming of the basic fabricated article  
in many instances is of significant economic importance.  
Usually the basic article, quite apart from the defective  
nickel deposit, represents considerable value in terms of  
labor and materials, and consequently if this can be sal-  
vaged in reusable form by removing the defective deposit,  
worthwhile economies can be effected.

There have been many compositions developed for  
stripping various plated deposits, including nickel, from  
their substrates. Some of these incorporate strongly acidic  
systems which attack the substrate as well as the nickel  
deposit which it is desired to remove. Others incorporate  
cyanide compounds which introduce health hazards. Still  
others involve waste liquor disposal problems. Many of  
the earlier systems also are rather slow in operation, are  
critical in respect to control of operating conditions and  
have rather limited capacity for dissolving nickel before  
they must be replenished or entirely replaced.

I have discovered improved compositions effective in  
stripping nickel deposits in aqueous solution which offer  
certain desirable features and advantages over the prior  
art. My system is completely alkaline and thus especially  
adapted to stripping of nickel from ferrous substrates  
which are rapidly attacked in acid environments employed  
in many of the stripping systems used heretofore. My sys-  
tem is operative in the presence of copper which very  
commonly is used as a flash or strike for nickel but which  
acts as a poison in some of the more effective prior strip-  
ping compositions, rendering them useless. My system  
avoids health hazards inherent in systems employing  
cyanide compounds used heretofore, being entirely free of  
cyanides in its make-up. My composition is inherently  
able to activate the nickel surface to be dissolved and to  
maintain a high rate of metal dissolution until the rate

2

determining component or components are consumed. One  
of the most important features of my composition is the  
high rate of nickel dissolution obtained at low, ambient  
temperatures, which drastically reduces evaporation losses  
and prolongs the useful life of the stripping system. An-  
other advantage of my system is that it presents no waste  
liquor disposal problems such as those encountered with  
cyanides and chromates, since the waste may be dis-  
charged as an effluent without treatment other than dilution  
if local authority permits nickel and copper in the  
effluent. If this is not permitted, these metals can very  
readily be precipitated from my system.

The composition is applicable to stripping nickel from  
the usual ferrous substrates, including those containing a  
flash deposit of copper as for example in automotive hard-  
ware or the like. It is also useful, of course, in stripping  
from non-metallic basis articles such as plastics and  
ceramics commonly used in electronic components as well  
as automotive applications.

20 The stripping compositions herein disclosed consist es-  
sentially of an oxidizer, a complexing agent for the nickel,  
a sulfur-containing activator for the nickel and, where  
necessary, a deactivator for copper to prevent copper  
poisoning of the stripping solution.

25 The oxidizers in my system are oxy-halogen com-  
pounds selected from the group consisting of the alkali and  
alkaline earth metal normal chlorites, hypochlorites,  
bromates and hypobromites. Sodium or potassium chlorites  
are preferred for reasons of availability and cost.

30 The nickel complexer may be the ammonium ion from  
aqueous ammonia or buffered as ammonium carbonate,  
chloride, fluoride, phosphate, sulfate, nitrate, or acetate  
salts; amines and substituted amines such as ethylenediamine,  
the disodium salt of ethylenediamine tetraacetic

35 acid; nitrilotriacetic acid and its salts, and amino acids  
such as glycine and its salts, e.g. sodium glycinate; the  
salts of glycolic acid, gluconic acid; and other hydroxy  
acids such as tataric. The inorganic ammonium salts are  
especially good from a cost standpoint. The amines on  
40 the other hand have the added advantage of lower volatil-  
ization losses.

As nickel activators, I use sulfur-containing compounds  
belonging to the groups comprising metallic sulfides, non-  
metallic sulfides, thioacids and their salts, aliphatic nitro-  
gen sulfur compounds and aromatic nitrogen sulfur com-  
pounds. In fact almost any organic or inorganic sulfur  
compound having at least limited solubility in aqueous  
solution is effective.

Finally, where a deactivator for copper is needed, I pre-  
fer to use diethyldithiocarbamic acid sodium salt, sub-  
stituted dithiocarbamates, thioanilides, and organic sulfur-  
containing carbamides.

55 In each of the foregoing categories, mixtures of the  
agents mentioned, rather than just a single agent, may  
be employed provided of course the mixture does not  
itself interact to destroy the effectiveness of the agents.

Solutions containing the foregoing combination of  
components are operative over a pH range of about 8.0  
60 to 13.0 and, where necessary, an amine is added to effect  
the desired degree of alkalinity within these limits. Gener-  
ally a pH of 8.5 to 10.5 is preferred.

65 The stripping solution is not critical as to concentration  
of oxidizer, nickel complexer, activator for the nickel  
or deactivator for the copper. Practically useful solutions  
are obtained when the oxidizer concentration is as little  
as 0.1 mol per liter up to near saturation. The complexer  
concentration is dependent upon the amount of nickel to  
be dissolved. The system is operative where the complexer  
is present at a mol ratio of at least 1:1 but for practical  
operation, more useful stripping speeds are obtained with  
a mol ratio preferably of 3:1 or greater. The amount of

the complexer needed may be determined from the amount of the oxidizer required to oxidize the elemental nickel deposit to be dissolved by converting it to the nickelous state. The activator is found to be effective in molar concentrations from trace amounts as little as 0.00023 to 0.23 mol per liter. The preferred concentration is about 0.0023. The copper deactivator is likewise found to be effective over a range of concentrations from about 0.008 to 0.2 mol per liter, preferably within the limits of solubility, or about 0.01 to 0.015 mol per liter. In some cases a single sulfur-containing compound may serve both as activator for nickel and as deactivator for copper, in which case the molar concentration should equal the sum of the concentrations of the separate components.

The temperature of the solution used in stripping nickel is not critical, and the system exhibits outstanding improvement over earlier systems at ambient room temperatures, making commercial operation practical under conditions which minimize evaporation losses and effect related advantages of economy and installation simplification.

In this system, in the process of activating the nickel surface by the sulfur-containing compounds, a film forms on the dissolving nickel or on the substrate. This film is essential for dissolution of the nickel but should be removed from the substrate before performing further plating or finishing operations. Such film or smut removal may be accomplished in any of several well known ways, or it can be effected in a solution of the same oxidizer and complexer, but without a nickel activator, used in the stripping bath itself.

Examples of typical solutions within the purview of the invention, and the stripping rates obtained by them, are as follows:

*Example 1*

The following solutions are useful in stripping nickel from a substrate where no copper is present:

|                             | Mol/l.                  | Mol/l.                  | Mol/l.                  |
|-----------------------------|-------------------------|-------------------------|-------------------------|
|                             | Mil/Min.<br>(At 25° C.) | Mil/Min.<br>(At 25° C.) | Mil/Min.<br>(At 25° C.) |
| Ammonia, aqua.....          | 4.50                    | 3.37                    | 2.25                    |
| Ammonium carbonate.....     | 2.25                    | 3.37                    | 4.50                    |
| Sodium chlorite.....        | 0.375                   | 0.375                   | 0.375                   |
| Ammonium thiocyanate.....   | 0.0023                  | 0.0023                  | 0.0023                  |
| Nickel stripping speed..... | 0.062                   | 0.058                   | 0.062                   |

Substitution of any of the anions named hereinabove for carbonate in the ammonium complexer is effective, and produces no significant change in stripping rate at the same mol concentrations. Likewise substitution may be made of other cations, such as potassium, lithium or calcium for example, in the oxidizer, again without change in molar concentration, and will be operative.

*Example 2*

Where copper is present as a strike under the nickel, the following system is effective:

|                                                       | Mol/l.         |
|-------------------------------------------------------|----------------|
| Ammonia, aqua.....                                    | 450.           |
| Ammonium carbonate.....                               | 2.25           |
| Sodium chlorite.....                                  | 0.375          |
| Ammonium thiocyanate.....                             | 0.0023         |
| Sodium diethyldithiocarbamate.....                    | 0.008 to 0.016 |
| Nickel stripping speeds,<br>(mil/min. at 25° C.)..... | 0.060.         |

*Example 3*

Compositions identical with those of Examples 1 and 2 except for the substitution of different complexers provide effective stripping also. For example, in place of the ammonia-ammonium carbonate, equal molar concentrations of ethylene-diamine may be employed. Providing also that the pH of the solution is maintained at the afore-

said level of 8.0 to 13.0, where necessary by the addition of aqueous ammonia or ethylene-diamine, other complexers such as disodium ethylenediamine tetraacetic acid, nitrilotriacetic acid, glycine or glycolic, gluconic and tartaric acids and their salts may likewise be used. The molar concentrations of these complexers, either singly or in combination, must of course be sufficient to provide the desired mol ratio of at least 1:1 and preferably higher in respect to the amount of nickel to be dissolved. One of the major advantages of the foregoing group of complexers is a lower volatility than the straight aqueous ammonia-ammonium salt compositions. Stripping rates are generally satisfactory although generally lower than in Example 1. The system is operative at a temperature as low as 15° C. but a preferred practical lower limit is around 25° C. for the system of Examples 1 and 2. Other systems, as noted hereinafter may require somewhat higher temperatures on the order of 50° to 75° C. to provide practical stripping speeds. Examples using other complexing agents than the ammonia-ammonium carbonate are given in Table 1.

TABLE 1

|                                            | Mol/l.   | Mol/l.   |
|--------------------------------------------|----------|----------|
|                                            | Mil/Min. | Mil/Min. |
| Ethylenediamine.....                       | 1.8      | 1.5      |
| Sodium glycinate.....                      | -----    | 0.375    |
| Sodium chlorite.....                       | 0.375    | 0.375    |
| Ammonium thiocyanate.....                  | 0.0023   | 0.0023   |
| pH.....                                    | 8.4      | 9.8-10   |
| Nickel stripping speed (at 70-75° C.)..... | 0.002    | 0.03     |

35 *Example 4*

In place of sodium chlorite in Examples 1 and 2, other oxidizers may also be used. Thus, other chlorite salts such as potassium, lithium or calcium are fully operative when substituted in equal molar concentrations. Still other oxidizers of the oxy-halogen group which are effective are the corresponding bromate salts and the hypobromites. The iodates and fluorates do not appear to be operable in this system. Again, typical nickel stripping rates for systems employing some of these other oxidizers are as follows:

TABLE 2

|                          | Mol/l.                     | Mol/l.                     |
|--------------------------|----------------------------|----------------------------|
|                          | Mil/Min.<br>(At 49-54° C.) | Mil/Min.<br>(At 25-27° C.) |
| Ammonia, aqua.....       | 4.0                        | 9.0                        |
| Ammonium carbonate.....  | 2.25                       | 4.45                       |
| Sodium hypochlorite..... | 0.375                      | -----                      |
| Sodium hypobromite.....  | -----                      | 0.75                       |
| Sodium thiocyanate.....  | 0.0023                     | 0.0023                     |
| pH.....                  | 9-10                       | 9-10                       |
| Nickel stripping.....    | 0.002                      | 0.0005                     |

55 *Example 5*

Nickel activators other than ammonium thiocyanate as given in Examples 1 and 2 includes such divalent sulfur ion-supplying compounds as sodium, potassium, ammonium, calcium, barium, magnesium, aluminum and hydrogen sulfides, and carbon disulfide. Organic nitrogen-sulfur compounds, both aliphatic and aromatic, are operative. For example, thioanilides and thiocarbamides, such as dimethyl- or diethyl-thiourea and the corresponding dithiocarbamic acids, and their salts, thioacetic acid and thioamide (e.g. thioacetamide) derivatives, are typical of useful aliphatic compounds. Correspondingly, aromatic nitrogen-sulfur compounds such as thiocarbanilide (diphenylthiourea) and phenyldithiocarbamic acid and its salts are operative. Again at the same molar concentra-

tions, the nickel stripping rates remain good with such activators.

TABLE 3

|                                                         | Mol/l. |
|---------------------------------------------------------|--------|
| Ammonia, aqua                                           | 4.0    |
| Ammonium carbonate                                      | 2.25   |
| Sodium chlorite                                         | 0.375  |
| Thiourea                                                | 0.023  |
| Nickel stripping speed<br>(mil/min. at 25° C.), 0.0137. |        |

*Example 6*

The organic activators mentioned in the preceding example may serve a dual function in the stripping system, in that not only are they effective for activating the nickel but they also serve as deactivators for copper where this is encountered, preventing poisoning of the system by the copper. For instance, in Example 2 above, ammonium thiocyanate may be omitted if the molar concentration of sodium diethyldithiocarbamate is at a level of about 0.01 or better.

*Example 7*

For practical purposes, a minimum molar concentration of the complexer in solution should be about 3:1 relative to the nickel. With this in mind it is sometimes advantageous to prepare a composition in the form of a concentrate for reducing transportation costs. In such a case, a solution having a make-up composition of complexer, oxidizer and activator mol ratio of around 3.0:0.3:0.003 is quite suitable. Where a combined activator-deactivator is used, the ratio should be 3.0:0.3:0.01. Preferably, a higher concentration of complexer in the bath is desirable but this can be conveniently added in the form of aqueous ammonia, ethylenediamine, etc. at the time of making up the actual solution to be used in the stripping process. The minimum pH of 8.0 must also be observed, of course.

*Example 8*

It is also possible to use ethylenediamine tetraacetic (EDTA) both as a nickel complexing agent and as a copper deactivator, but in such instance a sulfur-type nickel activator must also be present. While the EDTA might itself serve as the only nickel complexer in solution, this increases the expense and therefore it is more practical to use it in combination with ammonia or one of the ammonium salts such as the nitrate or sulfate. The molar concentrations of EDTA, either alone or in combination with an ammonium ion supplying component, should in this case equal the total of the molar concentrations recommended above for the complexer plus the copper deactivator. Since the latter requires only trace amounts to be effective, maintaining the molar concentration of the complexing agent (EDTA alone or in combination with others named) above the minimums recommended for the complexing agent alone will be sufficient.

As discussed above, one of the principal advantages of the systems herein disclosed is that they are operable in terms of practical commercial use where copper ions get into the stripping solution. This can and does occur, for example in the commonly encountered situation where there is, in addition to the nickel plate, a flash coating of copper on the substrate. This flash coating is on the order of 0.03 mil thick in a typical case, and is stripped along with the nickel in my solution. But the copper thus brought into solution does not poison the stripping bath so long as its concentration remains below a weight ratio of about 1:60 relative to nickel. The amount of copper in the usual flash coating is well below that needed to reach such a concentration. Thus my solution has the advantage of far higher stripping rates than cyanide and other alkaline solutions, and also avoids the health hazards of the cyanide systems.

What is claimed is:

1. A nickel stripping composition for use in aqueous solution, which consists essentially of:

(a) an oxidizer selected from the group consisting of the sodium, potassium, calcium and lithium salts of hypochlorite, normal chlorite, bromate and hypobromite;

(b) a nickel-complexing agent selected from the group consisting of ammonia and ammonium carbonate, chloride, fluoride, phosphate, sulfate, nitrate and acetate; ethylenediamine, ethylenediamine tetraacetic acid; nitrilotriacetic acid; glycine, glycolic, gluconic and tartaric acids and salts thereof; and

(c) a divalent sulfur ion-supplying compound as a nickel-activating agent, said compound being selected from the group consisting of sodium, potassium, calcium, barium, magnesium, aluminum, ammonium, hydrogen sulfides and carbon disulfide; thiocyanates, thioacetates, thioamides, thioanilides, thiocarbamides and the salts thereof;

5 said oxidizer being present in amount to provide in solution from about 0.1 mol per liter to near saturation; said complexing agent being present in a mol ratio of at least 1:1 relative to the nickel to be dissolved; and said activating agent being present in small but effective amount up to about 0.23 mol per liter.

2. A composition for selectively stripping nickel deposits from substrates on which they are plated, which composition is operative in the presence of copper ions in 10 the stripping solution and which consists essentially, in combination with the composition defined in claim 1, of a copper-deactivating agent selected from the group consisting of methyl, ethyl and phenyl substituted thioanilide and dithiocarbamide and the sodium, potassium and ammonium salts thereof, said copper-deactivating agent being present in small but effective amount up to about 0.23 mol per liter.

3. A composition for selectively stripping nickel deposits from substrates on which they are plated, which 15 composition is operative in the presence of copper ions in the stripping solution and consists essentially of:

(a) an oxidizer selected from the group consisting of the sodium, potassium, calcium and lithium salts of hypochlorite, normal chlorite, bromate and hypobromite;

(b) a nickel complexing agent selected from the group consisting of ammonia and ammonium carbonate, chloride, fluoride, phosphate, sulfate, nitrate and acetate; ethylenediamine; ethylenediamine tetraacetic acid; nitrilotriacetic acid; glycine, glycolic, gluconic and tartaric acids; and

(c) a nickel-activating, copper-deactivating divalent sulfur ion-supplying compound selected from the group consisting of thiocarbanilide, dimethyldithiocarbamic, diethyldithiocarbamic and phenyldithiocarbamic acids and salts thereof;

20 said oxidizer being sufficient to provide in solution at least 0.1 mol per liter to near saturation, said complexing agent being present in a mol ratio of at least 1:1 relative to nickel to be dissolved; and said nickel-activating, copper-deactivating agent being present in small but effective amount up to about 0.23 mol per liter.

4. A nickel stripping composition for use in aqueous solution which consists essentially of ammonium carbonate, sodium chlorite and ammonium thiocyanate in mol ratios of approximately 3.0:0.3:0.003.

5. A nickel stripping composition for use in aqueous solution which consists essentially of approximately 3 mols of ammonium carbonate, 0.3 mol sodium chlorite, and 0.01 mol sodium diethyldithiocarbamate.

6. A composition for use in aqueous solution in dissolving nickel deposits from substrates on which they are plated, which consists essentially, in addition to water, of an oxidizer selected from the group consisting of the sodium, potassium, calcium and lithium salts of chlorite,

hypochlorite, bromate and hypobromite; a nickel complexing agent selected from the group consisting of ethylenediamine, disodium ethylenediamine tetraacetic acid, nitrilotriacetic acid, glycine, glycolic, gluconic and tartaric acids; and a sulfur-containing nickel activating agent capable of providing divalent sulfur ions in solution; said oxidizer being present in amount to provide in solution from about 0.1 mol to near saturation, said complexing agent being present in a mol ratio of at least 1:1 relative to the nickel to be dissolved, and said nickel activating agent being present in small but effective amount up to about 0.23 mol per liter.

7. A composition for use in aqueous solution for dissolving nickel deposits from substrates on which they are plated, which consists essentially, in addition to water, of an oxidizer selected from the group consisting of the sodium, potassium, calcium and lithium salts of hypochlorite, normal chlorite, bromate and hypobromite; a nickel complexing agent selected from the group consisting of ethylenediamine, disodium ethylenediamine tetraacetic acid, nitrilotriacetic acid, glycine, glycolic, gluconic and tartaric acids; and a sulfur-containing nickel activating agent capable of providing divalent sulfur ions in solution; said oxidizer being present in amount to provide in solution from about 0.1 mol per liter to near saturation, said complexing agent being present in a mol ratio of at least 1:1 relative to the nickel to be dissolved, and said activating agent being present in small but effective amount up to about 0.23 mol per liter.

8. A composition as defined in claim 7, wherein the sulfur-containing nickel activating agent is selected from the group consisting of sulfide, thiocyanate, thioacetate, thioamide, thioanilid and thiocarbamide.

9. The method of dissolving metallic nickel deposits from articles having deposits thereof on their surfaces, which comprises subjecting the surface of the article to an aqueous solution consisting essentially, in addition to water, of:

- (a) an oxidizing agent in amount of from about 0.1 mol per liter to near saturation, selected from the group consisting of the sodium potassium, calcium, and lithium salts of hypochlorite, normal chlorite, bromate and hypobromite;
- (b) a nickel-complexing agent, in amount providing a mol ratio of at least 1:1 relative to the nickel to be dissolved, selected from the group consisting of ammonia and ammonium carbonate, chloride, fluoride, phosphate, sulfate, nitrate and acetate; ethylenediamine; ethylenediamine tetraacetic acid, nitrilotriacetic acid; glycine, glycolic, gluconic and tartaric acids and salts thereof; and
- (c) a divalent sulfur ion-supplying compounds as a nickel activating agent, in small but effective amount up to about 0.23 mol per liter, selected from the

group consisting of sodium, potassium, calcium, barium, magnesium, aluminum, ammonium, hydrogen sulfides and carbon disulfide; thiocyanates, thioacetates, thioamides, thioanilids, thiocarbamides and the salts thereof;

5 while maintaining said solution at temperatures ranging from approximately 15° to 75° C.

10. The method defined in claim 9 wherein copper ions may also be present in solution, which comprises subjecting the surface of the article to an aqueous solution as defined in claim 9 but also containing a small but effective amount up to about 0.23 mol per liter of a copper deactivating agent selected from the group consisting of the methyl, ethyl and phenyl substituted thioanilids and dithiocarbamides and the sodium, potassium and ammonium salts thereof.

15. The method defined in claim 9 wherein copper ions may also be present in solution, which comprises subjecting the surface of the article to an aqueous solution as defined in claim 9, wherein said nickel activator is present in amount of at least about 0.01 mol per liter and is selected from the group consisting of thiocarbanilide, dimethylthiocarbamic, diethylthiocarbamic and phenyl-dithiocarbamic acids and the sodium, potassium and ammonium salts thereof.

20. The method of dissolving metallic nickel deposits from articles having deposits thereof on their surfaces, which comprises subjecting the surface to an aqueous solution consisting essentially in addition to water of an oxidizer selected from the group consisting of the sodium potassium, calcium and lithium salts of chlorite, hypochlorite, bromate and hypobromite; a nickel complexing agent selected from the group consisting of ethylenediamine, disodium ethylenediamine tetraacetic acid, nitrilotriacetic acid, glycine, glycolic, gluconic and tartaric acid; and a sulfur-containing nickel activating agent capable of providing divalent sulfur ions in solution; said oxidizer being present in amount to provide in solution from about 0.1 mol to near saturation, said complexing 25 agent being present in a mol ratio of at least 1:1 relative to the nickel to be dissolved, and said nickel activating agent being present in small but effective amount up to about 0.23 mol per liter; while maintaining said solution at temperatures ranging from approximately 15° to 75° C.

#### References Cited

#### UNITED STATES PATENTS

|           |         |                 |       |           |
|-----------|---------|-----------------|-------|-----------|
| 2,561,065 | 7/1951  | Meyer           | ----- | 252—103 X |
| 3,102,808 | 9/1963  | Weisberg et al. | ----- | 252—364 X |
| 3,163,524 | 12/1964 | Weisberg et al. | ----- | 75—97 X   |

LEON D. ROSDOL, Primary Examiner.

M. WEINBLATT, Assistant Examiner.